

Dec. 28, 1971

C. J. EGAN

3,630,885

PROCESS FOR PRODUCING HIGH YIELDS OF LOW FREEZE POINT JET FUEL

Filed Sept. 9, 1969



INVENTOR

CLARK J. EGAN

BY Ray J. Davis

C. J. Torkin  
ATTORNEYS

1

3,630,885

## PROCESS FOR PRODUCING HIGH YIELDS OF LOW FREEZE POINT JET FUEL

Clark J. Egan, Piedmont, Calif., assignor to Chevron  
Research Company, San Francisco, Calif.  
Filed Sept. 9, 1969, Ser. No. 856,304  
Int. Cl. B01j 11/08; C10g 13/02, 37/02

U.S. CL. 208—59

10 Claims

### ABSTRACT OF THE DISCLOSURE

Process for obtaining a high yield of low freeze point jet fuel from a hydrocarbon feedstock containing materials boiling above the jet fuel boiling range and containing at least 5 volume percent normal paraffins which comprises subjecting said feedstock to hydrocracking and isomerization in the presence of hydrogen and a catalyst comprising alumina, a halogen and a component selected from the metals platinum, palladium and iridium and compounds of said metals, whereby the amount of jet fuel boiling range materials is increased and normal paraffins are isomerized, and selectively hydrocracking the remaining normal paraffins in the presence of hydrogen and a catalyst comprising mordenite in hydrogen form and at least one hydrogenating component.

This invention relates to jet fuel production, and more particularly to production of high yields of low freeze point jet fuel from hydrocarbon feedstocks containing materials boiling above the jet fuel boiling range.

### PRIOR ART

The necessity for jet fuels to be characterized by low freeze points is well known, and is reflected in all military and commercial jet fuel specifications. Many patents have been issued directed to various processes for producing low freeze point jet fuels, for example U.S. Patent 3,110,662. Said patent also indicates that it is known to hydrocrack hydrocarbon feedstocks containing materials boiling above the jet fuel boiling range, to produce jet fuels.

Catalytic dewaxing of hydrocarbon oils is well known in the art and refers to the reduction of the normal paraffin content of the oils by catalytic conversion of normal paraffins rather than by mere physical removal of normal paraffins without conversion thereof.

Copending Egan U.S. patent application Ser. No. 771,880 now U.S. Patent 3,539,495 adequately discusses the reasons for catalytic dewaxing of hydrocarbon oils, including reasons why continuing efforts are being made in the petroleum industry to find improved dewaxing catalysts and processes.

A recent development in the area of catalytic dewaxing is provided by accomplishing catalytic dewaxing with a catalyst comprising a crystalline aluminosilicate zeolite in hydrogen form having uniform pore openings with a minor pore diameter as determined by crystallography of not less than 5.8 and a major pore diameter less than 8 angstroms at a temperature of at least 450° F., as disclosed in Texaco Development Corporation South Africa Patent 67/3685, equivalent to U.S. Patent 3,539,458 issued Nov. 10, 1970. The zeolite having the required characteristics is a mordenite-type zeolite. It is highly preferable that the mordenite be in hydrogen form; the sodium form, for example, produces inferior dewaxing results. A catalytic material, suitably a Group VIII metal, preferably a platinum group metal, preferably is associated with the zeolite. The decationized mordenite-type zeolite structures have pore sizes sufficiently large to admit not only the straight-chain hydrocarbons which it is desired to selectively convert to lower molecular weight

2

materials, but also cyclic hydrocarbons; in contrast, the straight-chain hydrocarbons alone are selectively admitted to 5-angstrom molecular sieves, the pores of which quickly become saturated with waxy components, causing catalyst deactivation. Accordingly, the decationized mordenite zeolite structures have a greater capacity for sustained selective conversion of straight-chain components than do 5-angstrom molecular sieves. The mordenite-type zeolite has a chain-type zeolite structure in which a number of chains are linked together into a structural pattern with parallel sorption channels similar to a bundle of parallel tubes, in contrast with the three-dimensional structural lattices which are characteristic of molecular sieve zeolites such as Y-type faujasites. The mordenite-type zeolite dewaxing catalyst preferably comprises a Group VIII hydrogenating component, particularly nickel, platinum, palladium and rhodium, in an amount of 0.1 to 10 weight percent, calculated as metal. When the hydrogenating component is platinum or palladium, the recommended amount is 0.1 to 5.0 weight percent, preferably 0.5 to 2.5 weight percent. When the hydrogenating component is nickel, cobalt or iron, the recommended amount is 1 to 10 weight percent, preferably 1 to 5 weight percent. Hydrogen, in conjunction with the hydrogenating component of the catalyst, extends the life of the catalyst during catalytic dewaxing by preventing fouling of the pore openings of the catalyst. The catalyst may be preconditioned in hydrogen before use, at a temperature in the range 450° to 1000° F.

30 A mordenite-type zeolite in hydrogen form that is suitable for purposes of the process of said South Africa Patent 67/3685 and for purposes of the present invention is the calcined synthetic "Zeolon H" mordenite sold commercially by the Norton Company.

35 As used hereinafter, the terms "mordenite," "hydrogen mordenite," and "mordenite in hydrogen form" are intended to include those mordenite-type zeolites indicated by said South Africa Patent 67/3685 to be desirable as catalytic dewaxing catalysts or as components of catalytic dewaxing catalysts.

### OBJECTS

40 In view of the continuing need for improvements in methods for producing high yields of low freeze point jet fuels from hydrocarbon feedstocks, and in view of the catalytic dewaxing advances disclosed in said South Africa Patent 67/3685, it would be desirable if a combination process were available for converting to low freeze point jet fuel in high yields a hydrocarbon feedstock unsuitable as jet fuel because of an unacceptably high end point and an unacceptably high normal paraffin content, which process would utilize said advances disclosed in said South Africa patent.

### DRAWING

45 The above and additional objects of the present invention, and the ways in which these objects are achieved, will better be understood from the following description when read in connection with the accompanying drawing, which is a diagrammatic illustration of apparatus and flow paths suitable for carrying out certain embodiments of the invention.

### STATEMENT OF INVENTION

50 In accordance with the present invention there is provided a process for producing a jet fuel which comprises contacting a hydrocarbon feedstock boiling in the range 450° to 750° F. and containing at least 5 weight percent, preferably 5 to 40 weight percent, more preferably at least 10 weight percent, and still more preferably 10 to 30 weight percent, normal paraffins in a first reaction zone with hydrogen and a hydrocracking-isomerization catalyst comprising alumina, a halogen, and a component

selected from the metals platinum, palladium and iridium and compounds of said metals, at hydrocracking-isomerization conditions including a temperature in the range 700° to 900° F., preferably 750° to 850° F., a pressure in the range of 500 to 3000 p.s.i.g., preferably 1000 to 2500 p.s.i.g., a liquid hourly space velocity in the range 0.1 to 10 volumes of said feedstock per volume of catalyst per hour, and a total hydrogen rate of 200 to 20,000 s.c.f., preferably 2000 to 8000 s.c.f., of hydrogen per barrel of said feedstock, and at a per-pass cracking conversion of said feedstock not more than 30 weight percent, preferably 5 to 30 weight percent, to products boiling below the initial point of said feedstock, with accompanying isomerization of normal paraffins to iso-paraffins, and catalytically dewaxing at least a portion of the effluent from said first reaction zone in a second reaction zone by contacting said portion with hydrogen and a dewaxing catalyst comprising mordenite in hydrogen form and at least one hydrogenating component, at catalytic dewaxing conditions including a temperature in the range 400° to 900° F., preferably 550° to 750° F., a pressure in the range of 100 to 2500 p.s.i.g., preferably 400 to 2000 p.s.i.g., a liquid hourly space velocity of 0.2 to 25 volumes of said feedstock per volume of catalyst per hour, and a total hydrogen rate of 200 to 20,000 s.c.f., preferably 2000 to 8000 s.c.f., of hydrogen per barrel of said feedstock, to produce a dewaxed product.

In a preferred embodiment said portion of the effluent from said first reaction zone that is dewaxed in said second reaction zone boils in the range 450 to 750° F., more preferably 450° to 600° F., contains less than 50 parts per million organic nitrogen, preferably less than 5 parts per million organic nitrogen and less than 100 parts per million organic sulfur, preferably less than 50 parts per million organic sulfur, and contains a substantially smaller weight percentage of normal paraffins than is contained in the portion of the hydrocarbon feedstock having the same boiling range. Despite certain language tending to teach to the contrary in said South Africa Patent 67/3685, better results are obtained if the nitrogen and sulfur contents of the hydrocarbon feed to the second reaction zone are kept within the above limits.

In accordance with a further embodiment of the process of the present invention a fraction boiling below 450° F. is removed from the effluent from said first reaction zone and the portion of the effluent from said first reaction zone that is catalytically dewaxed in said second reaction zone boils above 450° F., preferably in the range 450° to 600° F. The portion of the effluent from said first reaction zone that boils above 600° F. may be recycled to said first reaction zone.

In a further embodiment of the process of the present invention said first reaction zone and said second reaction zone are located in a single reactor pressure shell, and said hydrocarbon feedstock contains less than 10 parts per million organic nitrogen and less than 50 parts per million organic sulfur. When said first reaction zone and said second reaction are not located in a single reactor pressure shell, the feedstock supplied to the first reaction zone may contain more than 10 parts per million organic nitrogen and more than 50 parts per million organic sulfur, and the effluent from said first reaction zone may be hydrofining to reduce the organic nitrogen content thereof to less than 10 parts per million and the organic sulfur content thereof to less than 50 parts per million, prior to supplying the hydrofining material to said second reaction zone.

The halogen contained in said catalyst in said first reaction zone preferably is present as combined halogen, that is, in combination with at least one other component of the catalyst. The halogen preferably is selected from fluorine and chlorine, and therefore preferably is present as a halide selected from fluorides and chlorides. For example, fluorine may be combined with the alumina component of the catalyst to form aluminum fluoride. The halo-

gen may be present in an amount of 0.01 to 5.0 weight percent, calculated as halogen and based on the total catalyst.

The catalyst in the first reaction zone and the catalyst in the second reaction zone each advantageously may contain rhenium or a compound of rhenium, in an amount of 0.2 to 1.5 weight percent, calculated as metal and based on the total catalyst.

Each component selected from the metals platinum, palladium, iridium and compounds of said metals, that is present in the catalyst in the first reaction zone may be present in an amount of 0.2 to 1.5 weight percent, calculated as metal and based on the total catalyst.

The dewaxing catalyst in the second reaction zone, which comprises mordenite and at least one hydrogenating component, desirably will contain a Group VIII metal or metal compound hydrogenating component, preferably selected from the metal platinum, palladium, iridium, ruthenium, rhodium and nickel and compounds of said metals. Said dewaxing catalyst advantageously further may comprise carbon in an amount of at least 0.5 weight percent, based on the total catalyst. The carbon content of the catalyst may be obtained by contacting the catalyst with hydrogen and a heavy hydrocarbon distillate boiling in the range 500° to 1100° F., at a temperature in the range 400° to 900° F., a pressure in the range 500 to 3500 p.s.i.g., and a liquid hourly space velocity in the range 0.1 to 10, at a total hydrogen rate in the range 200 to 20,000 s.c.f. of hydrogen per barrel of said distillate, until the catalyst contains the desired amount of carbon. It has been found that the presence of the carbon in the catalyst makes the catalyst more selective for cracking normal paraffins, and therefore makes the catalyst a more efficient dewaxing catalyst.

The amount of the hydrogenating component present in the catalyst in the second reaction zone is discussed under prior art, above.

#### DISCUSSION OF DRAWING

Referring now to the drawing, there is shown in a diagrammatic illustration of apparatus and flow paths suitable for carrying out the process of one embodiment of the present invention.

A hydrocarbon feedstock boiling in the range 450° to 750° F. and containing at least 5 weight percent normal paraffins is supplied through line 1 to hydro-cracking-isomerization zone 2, which is supplied with hydrogen through line 3. Said feedstock is hydrocracked and isomerized in zone 2 in the presence of a halogen-containing catalyst as previously described and at conditions previously described. The effluent from zone 2 is passed through line 4 to separation zone 5, which may be a distillation zone, and is there separated into fractions, including:

(1) A C<sub>4</sub>- fraction which is withdrawn through line 6;

(2) A 450° F.— fraction which is withdrawn through line 7;

(3) A fraction boiling in the range 450° to 600° F. which is passed through line 8 to dewaxing zone 9;

(4) A 600° to 750° F.— fraction which is recycled from zone 5 to zone 2 through line 10.

The fraction entering zone 9 through line 8 is catalytically dewaxed in zone 9 in the presence of hydrogen entering zone 9 through line 11 and in the presence of the mordenite-containing dewaxing catalyst previously described, at the catalytic dewaxing conditions previously described. The effluent from zone 9, reduced in normal paraffin content compared with the fraction in line 8, is recovered from zone 9 through line 12 for use in part or in its entirety as a superior, low freeze point jet fuel. Said fraction may be further hydrogenated in a conventional manner, if desired, to further improve the smoke point thereof.

The hydrocarbons supplied to zone 9 through line 8 preferably have a limited nitrogen content and sulfur content, as previously described. This limited nitrogen

content and sulfur content may be a result of already adequately low nitrogen and sulfur levels in the hydrocarbons in line 1 because of prior hydrofining or otherwise, or may be a result of subjecting the hydrocarbons in line 4 or line 8 to a separate, conventional hydrofining treatment.

## EXAMPLES

The following examples will serve to further illustrate the process of the present invention.

## Example 1

A hydrocarbon feedstock was subjected to catalytic isomerization and then to catalytic dewaxing in accordance with the process of the present invention. The hydro-isomerization catalyst was in the form of a fixed bed located within a reactor pressure shell above a fixed bed of the catalytic dewaxing catalyst located within the same reactor pressure shell. Each catalyst was present in an amount of 50 volume percent of the total catalyst in the reactor shell. The hydrocarbon feedstock and hydrogen were introduced into the reactor shell at the top, and a liquid product was removed from the bottom of the reactor shell. Details of the operation were as follows:

## A. Hydrocarbon feedstock:

## ASTM D-86 distillation:

|                                |         |
|--------------------------------|---------|
| ST/10%                         | 485/508 |
| 50%                            | 521     |
| 90%/EP                         | 542/560 |
| Gravity, ° API                 | 33.3    |
| Organic sulfur, p.p.m.         | <10     |
| Organic nitrogen, p.p.m.       | 0.29    |
| Freeze point, ° F.             | +7      |
| Pour point, ° F.               | -20     |
| Aniline point, ° F.            | 157     |
| Paraffins, vol. percent        | 24.6    |
| Naphthenes, vol. percent       | 67.0    |
| Aromatics, vol. percent        | 8.4     |
| Naphthalenes, vol. percent     | 0.6     |
| Smoke point, mm.               | 19/18   |
| Normal paraffins, wt. percent: |         |
| C <sub>14</sub>                | 5.2     |
| C <sub>15</sub>                | 0.6     |
| C <sub>16</sub>                | 1.1     |
| C <sub>17</sub>                | 1.9     |
| C <sub>18</sub>                | 1.2     |

| B. Operating conditions                                                      | Isomerization catalyst<br>(upper bed) | Dewaxing catalyst<br>(lower bed) |
|------------------------------------------------------------------------------|---------------------------------------|----------------------------------|
| Temperature, ° F.                                                            | 800                                   | 645                              |
| Pressure, p.s.i.g.                                                           | 2,100                                 | 2,100                            |
| LHSV, V./V.hr.                                                               | 3.0                                   | 3.0                              |
| Total hydrogen rate, s.c.f. of hydrogen per barrel of hydrocarbon feedstock. | 5,000                                 | 15,000                           |

<sup>1</sup> Adjusted by effect of reaction in upper bed.

| C. Catalysts               | Isomerization catalyst                                                                                                                        | Dewaxing catalyst                                                               |
|----------------------------|-----------------------------------------------------------------------------------------------------------------------------------------------|---------------------------------------------------------------------------------|
| Hydrogenating component(s) | {Platinum <sup>1</sup> ...<br>Rhenium <sup>2</sup> ...<br>Alumina <sup>3</sup> ...<br>Fluoride <sup>4</sup> ...<br>Chloride <sup>5</sup> ...} | {Palladium <sup>6</sup> ...<br>Mordenite, <sup>7</sup> ...<br>in hydrogen form. |
| Other component(s)         |                                                                                                                                               |                                                                                 |

<sup>1</sup> 0.37 weight percent of total catalyst.

<sup>2</sup> 0.35 weight percent of total catalyst.

<sup>3</sup> Approximately 98.5 weight percent of total catalyst.

<sup>4</sup> 0.5 weight percent of total catalyst, calculated as F.

<sup>5</sup> 0.22 weight percent of total catalyst, calculated as Cl.

<sup>6</sup> 2.0 weight percent of total catalyst.

<sup>7</sup> 98.0 weight percent of total catalyst.

## 6

## D. Product distribution, weight percent:

|                                |       |
|--------------------------------|-------|
| C <sub>1</sub> +C <sub>2</sub> | 0.5   |
| C <sub>3</sub>                 | 2.0   |
| iC <sub>4</sub>                | 2.5   |
| nC <sub>4</sub>                | 1.5   |
| iC <sub>5</sub>                | 1.5   |
| nC <sub>5</sub>                | 1.3   |
| iC <sub>6</sub>                | 1.0   |
| nC <sub>6</sub>                | 0.7   |
| C <sub>7</sub> -300° F.        | 3.5   |
| 300° F.+                       | 85.5  |
| Total                          | 100.0 |

E. Yield of 300° F.+ product based on hydrocarbon feed, weight percent

15 85.5

## F. Characteristics of 300° F. plus product:

|                     |           |
|---------------------|-----------|
| Boiling range, ° F. | 300-575   |
| Gravity, ° API      | 35.1      |
| Aniline point       | 154       |
| Smoke point, mm.    | 18        |
| Freeze point, ° F.  | below -94 |

## Example 2

25 The operation of Example 1 is repeated, using an additional portion of the same feedstock, at the same conditions except that the temperature in the upper bed is 550° F. rather than 800° F., so that the first bed serves merely to hydrogenate the feedstock rather than to cause hydrocracking and isomerization of any appreciable amount of the normal paraffins therein.

Because the mordenite catalyst alone does not lower the boiling range of the feed sufficiently to meet jet fuel specifications, only the lower-boiling 75 volume percent of the 300° F.+ product is suitable for blending into jet fuel. The final yield of jet fuel is 0.75×92 weight percent, or 69 weight percent, of product having a freeze point of -61° F.

What is claimed is:

40 1. A process for producing a jet fuel which comprises contacting a hydrocarbon feedstock boiling in the range 450° to 750° F. and containing at least 5 weight percent normal paraffins in a first reaction zone with hydrogen and a hydrocracking-isomerization catalyst comprising alumina, a halogen, and a component selected from the metals platinum, palladium and iridium and compounds of said metals, at hydrocracking-isomerization conditions including a temperature in the range 700° to 900° F., a pressure in the range 500 to 3000 p.s.i.g., a liquid hourly space velocity in the range 0.1 to 10 volumes of said feedstock per volume of catalyst per hour, and a total hydrogen rate of 200 to 20,000 s.c.f. of hydrogen per barrel of said feedstock, and at a per-pass cracking conversion of said feedstock not more than 30 weight percent to products boiling below the initial boiling point of said feedstock, with accompanying isomerization of normal paraffins to isoparaffins, and catalytically dewaxing at least a portion of the effluent from said first reaction zone in a second reaction zone by contacting said portion with hydrogen and a dewaxing catalyst comprising synthetic mordenite in hydrogen form and at least one hydrogenating component, at catalytic dewaxing conditions including a temperature in the range 400° to 900° F., a pressure in the range 100 to 2500 p.s.i.g., a liquid hourly space velocity of 0.2 to 25 volumes of said feedstock per volume of catalyst per hour, and a total hydrogen rate of 200 to 20,000 s.c.f. of hydrogen per barrel of said feedstock, to produce a dewaxed product.

60 2. A process as in claim 1, wherein said feedstock contains at least 10 weight percent normal paraffins.

65 3. A process as in claim 1, wherein said portion of the effluent from said first reaction zone that is dewaxed in said second reaction zone boils in the range 450° to 750° F., contains less than 10 parts per million organic nitrogen and less than 50 parts per million organic sulfur, and

70 75

contains a substantially smaller weight percentage of normal paraffins than are contained in the portion of said hydrocarbon feedstock having the same boiling range.

4. A process as in claim 3, wherein said portion of the effluent from said first reaction zone that is dewaxed in said second reaction zone boils in the range 450° to 600° F.

5. A process as in claim 1, wherein said first reaction zone is operated at a per-pass cracking conversion of said feedstock in the range 5 to 30 weight percent of products boiling below the initial boiling point of said feedstock, and wherein a fraction boiling below 450° F. is removed from the effluent from said first reaction zone and wherein said portion of the effluent from said first reaction zone that is catalytically dewaxed in said second reaction zone boils above 450° F.

6. A process as in claim 1, wherein a portion of the effluent from said first reaction zone that boils above 600° F. is recycled to said first reaction zone and wherein the portion of the effluent from said reaction zone that is catalytically dewaxed in said second reaction zone boils in the range 450° to 600° F.

7. A process as in claim 1, wherein said first reaction zone and said second reaction zone are located in a single reactor pressure shell, and wherein said hydrocarbon feed-

stock contains less than 50 parts per million organic nitrogen and less than 100 parts per million organic sulfur.

8. A process as in claim 1 wherein said isomerization catalyst further comprises rhenium or a compound of rhenium.

9. A process as in claim 1, wherein said halogen is fluorine.

10. A process as in claim 1, wherein said dewaxing catalyst further comprises at least 0.5 weight percent carbon, based on the total catalyst.

#### References Cited

##### UNITED STATES PATENTS

|           |         |                 |       |         |
|-----------|---------|-----------------|-------|---------|
| 3,127,339 | 3/1964  | Scott           | ----- | 208—112 |
| 3,132,087 | 5/1964  | Kelley et al.   | ----- | 208—60  |
| 3,259,564 | 7/1966  | Kimberlin       | ----- | 208—111 |
| 3,395,096 | 7/1968  | Gladrow et al.  | ----- | 208—111 |
| 3,438,887 | 4/1969  | Morris          | ----- | 208—87  |
| 3,516,925 | 6/1970  | Lawrence et al. | ----- | 208—111 |
| 3,539,498 | 11/1970 | Morris et al.   | ----- | 208—111 |

DELBERT E. GANTZ, Primary Examiner

G. E. SCHMITKONS, Assistant Examiner

U.S. Cl. X.R.

208—66, 111, 112